

Apr. 3, 1923.

1,450,217

H. S. MARSH ET AL

METHOD OF AND APPARATUS FOR RECLAIMING SPENT PICKLING SOLUTION

Filed Aug. 3, 1921

2 sheets-sheet 1

FIG. I.



FIG. II.



WITNESSES

J. Herbert Bradley.  
Harry Vandervyde.

INVENTORS

Henry S. Marsh  
Ralf S. Cochran  
Key Christy and Christy  
their attorneys

Apr. 3, 1923.

1,450,217

H. S. MARSH ET AL

METHOD OF AND APPARATUS FOR RECLAIMING SPENT PICKLING SOLUTION

Filed Aug. 3, 1921

2 sheets-sheet 2



Patented Apr. 3, 1923.

1,450,217

# UNITED STATES PATENT OFFICE

HENRY S. MARSH AND RALF S. COCHRAN, OF YOUNGSTOWN, OHIO.

METHOD OF AND APPARATUS FOR RECLAIMING SPENT PICKLING SOLUTION.

Application filed August 3, 1921. Serial No. 489,545.

To all whom it may concern:

Be it known that we, HENRY S. MARSH and RALF S. COCHRAN, residing at Youngstown, in the county of Mahoning and State 5 of Ohio, citizens of the United States, have invented or discovered certain new and useful Improvements in Methods of and Apparatus for Reclaiming Spent Pickling Solution, of which improvements the following 10 is a specification.

Our invention relates to methods of and apparatus for the treatment of liquids burdened with salts in solution, with the end in view of separating the salt from its solvent. The invention, though not in its broader aspect so limited, finds primary application in the removal from spent pickling solutions used in metal-working mills and factories their burden of metallic salt, and so 15 reclaiming them for repeated service in the pickling operation. The ends in view are economy in the metal-treating operation, and regarding the industry in its relation to the community at large, the rectification and 20 salvage of an undesirable and deleterious by-product. The invention constitutes an improvement upon our prior inventions, described and claimed in Letters Patent of the 25 United States, Reissue No. 15,119, granted 30 us originally February 22, 1921, and reissued June 7, 1921, and in a pending application of ours, Serial No. 432,952, filed December 24, 1920.

Apparatus in which and in the operation 35 of which our present invention will be found, is illustrated in the accompanying drawings. Fig. I is a view in plan from above of apparatus of one particular form; Fig. II is a view in side elevation of a portion of the 40 apparatus of Fig. I; Fig. III is a diagrammatic showing of another form of apparatus. As presently will appear, the invention is present in both forms, and other variant forms will readily present themselves to the 45 mind of the trained engineer.

The method disclosed in our earlier applications alluded to is a method wherein the spent pickling solution (the substance primarily in contemplation) is caused to flow 50 in a looped conductor, the two branches of the loop being in heat-exchanging relation one to the other, a cooling agent is brought to bear upon the flowing stream in the loop of the circuit, and the salt, precipitated by 55 cooling, is allowed to separate by gravity from the stream as it flows. The so sep-

arated precipitate is, according to our earlier disclosures withdrawn from the stream, mingled necessarily with an appreciable quantity of the mother liquor, and, according to the disclosure of the later of our two applications above mentioned, the withdrawn material is carried to a centrifuge. In the centrifuge the mother liquor is separated from the salt, and from the centrifuge the 60 separated mother liquor is returned to the flowing stream first mentioned.

According to the method as now improved, there is no initial gravitational separation of precipitated salt from the great body of 70 the flowing stream. To the contrary precipitate and liquid are carried forward together, under conditions which diminish to the utmost the possibility of gravitational separation, and the whole is introduced into the 75 centrifuge. From the centrifuge the whole volume of liquid emerges and enters thence the return branch of the loop. The gain is simplification of apparatus and of operation. 80

There are incidental features modifying the operation as heretofore disclosed, and these features will become apparent as description proceeds.

Referring first to Fig. I of the drawings, 85 four concentrically arranged spiral coils are shown, bearing consecutively the reference numerals 1, 2, 3, 4. The fourth and innermost of these coils is in Fig. II shown, detached for simplification from the rest, in 90 side elevation. Each coil is double, consisting of two concentrically arranged pipes, and thus two passageways are formed, adapted to carry oppositely flowing streams, separated one from another by the walls of 95 the inner pipe, and thus in heat-interchanging relation, one to the other. The inner pipe is formed of acid-resisting material; it is continuous, through all the coils, from the approach 5 to the outermost coil to the escape 6 from the innermost. It is preferably formed of seamless copper tubing of the thinnest stock practicable, and any necessary joints are preferably formed by welding. The structure in view is a conveyor 100 through whose walls heat may pass by conduction most readily, smooth within, and uniform in bore from end to end, in order that the flowing stream may advance in uninterrupted sweep, without swirl or eddy. 105 The outer pipe of each coil must be strong to withstand pressure; it also will be formed

of acid-resisting material. Conveniently, it may be formed of lead; again, it may advantageously be formed of heat-insulating material suitably strengthened and rendered water-tight, and acid-resistant, either by lead lining, glazing, or otherwise.

The outer passageways of the several coils are not connected all of them in series as the inner passageways are connected, to 10 form a single continuous conveyor. As shown, the outer passageways of coils 3 and 1 are so connected, through the connecting pipe 7; but the outer passageway of coil 2 is connected at opposite ends with leads 8 15 and 9, and the outer passageway of coil 4 is similarly connected with leads 10 and 11. The reclaimed acid (reclaimed in the manner presently to be described) flows through lead 12 and gains access to the outer passageway 20 of coil 3, after traversing that passageway from end to end, this stream of reclaimed acid passes through pipe 7 to the outer passageway of coil 1, and, traversing that passageway from end to end, enters lead 13, 25 through which it flows to the pickling vat or to a suitable place of storage. Through the outer passageway of coil 2 a suitable cooling fluid circulates, and, as noted on the drawing, cold water is a suitable fluid, when 30 the pickling solution from iron or steel pickling is under treatment. Through the outer passageway of coil 4 another cooling fluid circulates. We have noted on the drawing that a suitable cooling fluid here is ammonia, 35 and this it will be understood is the cooling medium of a suitable refrigerating apparatus.

The mechanical unions of inner and outer tubes of the several coils may conveniently 40 be made by welding.

Lead 6 carries the material under treatment to separating apparatus, conveniently a centrifuge; lead 12 brings back reclaimed acid from the apparatus last mentioned.

45 Operation will readily be understood. Spent pickling solution flowing from the pickling vat or from a place of storage enters at a temperature of 150° F. say, through lead 5, the inner tube of coil 1; traversing that it passes in what is really a continuous conduit through the inner tube 50 of each coil, and advances finally through lead 6 to the separating apparatus (not shown in Fig. I). Reclaimed acid, returning through lead 12, traverses the outer pipe 55 of coils 3 and 1 successively, and passes on finally through lead 13 to a pickling vat again, or perhaps to a storage tank. Thus it will be seen that the stream from its entrance through lead 5 into the apparatus to 60 its exit through lead 13 is looped upon itself, and that, as in the disclosures of our earlier specifications the two branches of the loop are arranged in heat-exchanging relative 65 positions.

In the loop (or, to speak more specifically, in the innermost coil 4) the flowing stream is exposed to the cooling effect of the ammonia circulating in the outer pipe of this coil. This also, so far as method is concerned, presents no departure from our earlier disclosures. We have, however, so far modified the method of cooling that the entering stream, before reaching the loop of the circuit is exposed, not as in the earlier 70 case continuously to the cooling effect of the outflowing stream of reclaimed acid, but is exposed alternately, first to the cooling effect of the stream of reclaimed acid, then (in coil 2) to the cooling effect of a circulating stream of cold water, then again to the stream of reclaimed acid, at a point higher 75 up in that stream, where the reclaimed acid is cooler, and then at length it reaches the 80 loop of the circuit.

85 Another difference is to be noted between the apparatus and methods of our earlier applications and this: In those the precipitated salt was separated from the stream and sent separately to the centrifuge; here the whole stream goes to the separating apparatus.

90 Recurring to the progress of the material through the apparatus, it is to be remarked that, because of the presence of the two bodies of cooling media circulating in the outer pipes of coils 2 and 4 the inflowing stream is cooled as it advances, and that proportionately as it is cooled the outflowing stream as it traverses coils 3 and 1 is heated again. The spent acid enters as has been said at a temperature of 150°, more or less. In coil 1 it comes into heat-exchanging relation with the outflowing stream of reclaimed acid which reaches coil 1 at a temperature of say 40°. In consequence of heat interchange the advancing stream of entering spent acid passes from coil 1 to coil 2 at a temperature of 80°, more or less. In coil 2 the advancing stream is by heat transfer to the cooling medium there circulating reduced still further in temperature, to approximately 60°. In coil 3 there is further heat exchange with the outflowing stream of reclaimed acid, in consequence of 100 which the inflowing stream is reduced in temperature to approximately 40°. The loop of the circuit is now reached, and now as the inflowing stream advances through coil 4 it is by heat interchange with the refrigerating medium there encountered, reduced to approximately 30°. From coil 4 the material under treatment flows to the separating apparatus, and from the separating apparatus the reclaimed acid returns at substantially unchanged temperature to the outer pipe of coil 3. When it reaches coil 3 the loop of the circuit is completed. In coil 3 the outflowing reclaimed acid is warmed 105 from a temperature of approximately 30° 110 115 120 125 130

to 40°; it flows from coil 3 to coil 1, and in coil 1 is further warmed to approximately 130°, at which temperature it passes from the apparatus, to enter the pickling vat directly, or perhaps a storage tank.

Returning now to the progress of the material under treatment, it is cooled in its advance through the inner tube of the successive coils from its initial temperature of 10 150° more or less gradually to and slightly beyond the freezing point of water. As this point is reached the far greater part of the dissolved copperas is precipitated, and, being precipitated from a flowing stream, it 15 is precipitated in the condition of small and finely divided crystals. In consequence of the fact that the stream flows constantly and uniformly and without pockets or eddies, the precipitated crystals are swept along to 20 the separating apparatus. In that apparatus the precipitated crystals are removed, and by their removal reclaimed acid remains. This reclaimed acid, returning through the apparatus takes up heat again.

25 The heat economies are, with recognition of the modification due to the presence of the cooling medium in coil 2, essentially such as we in our earlier inventions have contemplated. The particular temperatures named 30 in the foregoing description are given in illustrative and exemplary sense; manifestly there may be considerable variation and departure from the actual figures given.

The elimination of the step of gravitational separation of the precipitated salt from the flowing stream, before introducing it to the centrifuge or equivalent apparatus, is a simplification; our perception that the whole body of material under treatment may pass 40 through the centrifuge is an invention that makes for economy. The refinement of using a second cooling medium, active on the inflowing branch of the looped stream of material is a refinement which we find 45 makes for efficiency. It will be realized that the temperature of this cooling medium is variable under the control of the user.

We have used the expressions "loop formed course" and "loop of the circuit," and 50 shall use them in the ensuing claims. That the course of the flowing stream is loop formed, is manifest; that the two branches of the loop are in heat-interchanging relationship, is manifest. By the expression 55 "the loop of the circuit" we mean to designate that portion of the course of the flowing stream which lies between the exit from the inner pipe of coil 3 to the entrance to the outer pipe of the same coil. That is to 60 say, from point *m*, Fig. I, to point *n*. In this interval the stream advances through the inner pipe of coil 4, through lead 6, through the separating apparatus, and through lead 12.

65 Fig. III serves to illustrate the fact that

the helical shape and the nesting together in concentric assembly of the several heat-exchanging units, are mere matters of convenience. Here, in place of four coils, four straight-away lengths of double pipe, 1<sup>a</sup>, 70 2<sup>a</sup>, 3<sup>a</sup>, and 4<sup>a</sup> are shown. Here also are shown diagrammatically, refrigeration apparatus for the heat-exchanger 4<sup>a</sup>, and a centrifuge. Additionally, a settling tank is indicated, into which the reclaimed acid may 75 pass from the centrifuge and before it begins its return flow; and also a pump is diagrammatically indicated, by means of which circulation may be maintained. In this case, the inflow is indicated to be gravitational, and the return to be effected by the pump; but, as will be perceived, this is a matter of engineering contrivance, and different arrangements will be made under 80 different circumstances. Fig. III shows 85 also a valve-controlled lead 14 from the water supply to the pipe 7 which conveys the returning reclaimed acid from heat-exchanger 3<sup>a</sup> to 1<sup>a</sup>. It is manifest that the removal of the salts, effected in the centrifuge (and copperas contains a large content of water of crystallization), must diminish the volume of the stream, so that, but for augmentation, the outflow must be 90 less than the inflow. Furthermore, in consequence of the addition in the pickling vat of fresh acid as the solution continues in service, it does practically come about that the reclaimed acid is often stronger than is required. For such reasons it may be found 100 desirable to introduce water into the out flowing stream in such manner and under such conditions of control as are indicated. Otherwise than now indicated, the correspondence of the showing of Fig. III to 105 that of Fig. I will be apparent on comparison, and manifestly, the mode of operation, wherein lies our invention so far as concerns method, is, with the detail explained, identically the same.

We claim as our invention:

1. The method herein described of removing from a solvent its burden of salt which consists in causing the solvent, laden initially with the dissolved salt, to flow in a 115 looped circuit, with the branches of the circuit in heat-exchanging relationship one to the other, cooling the flowing stream in the loop of the circuit to a temperature lower than the point of salt precipitation, and 120 causing the entire stream after such cooling and before entering the return branch of the circuit to undergo the operation of a centrifuge.

2. The method herein described of removing from a solvent its burden of salt which consists in causing the solvent, laden initially with the dissolved salt, to flow in a looped circuit, with the branches of the circuit in heat-exchanging relationship one 125 130

- to the other, cooling the stream at a point intermediate the length of the inflowing branch of the circuit, cooling the stream a second time in the loop of the circuit and 5 to a temperature lower than the point of salt precipitation, and after such separate cooling and before the flowing stream enters the return branch of the circuit, separating from the stream the precipitated salt.
- 10 3. The method herein described of removing from a solvent its burden of salt which consists in causing the solvent, laden initially with the dissolved salt, to flow in continuous stream, causing a stream of water 15 in part to flow in heat-exchanging relation to the flowing stream of solvent at a higher point in the course thereof, and in part to mingle with the flowing stream of solvent at a lower point in the course thereof, and in 20 separating from the stream of solvent at an intermediate point the burden of salt.
4. The method herein described of reclaiming spent pickling solution which consists in causing the spent solution, while still 25 retaining the heat of the pickling operation, to enter and having entered to flow in continuous stream and in its entirety through a loop-formed course, the branches of the stream being in heat-exchanging relation- 30 ship, one to the other, and through a centrifuge arranged in the turn of the course, and in colling the flowing stream on the intake side of the centrifuge to a temperature lower than the point of salt precipitation.
- 35 5. In apparatus for unburdening a solvent of its load of salt, a loop-formed conduit, the branches of the loop separated by a wall through which heat may pass from the stream flowing in one branch to the stream 40 flowing in the other, a centrifuge in the loop of the circuit into which and from which the entire stream flows, and means for cooling the flowing stream on the inflow side of the centrifuge, substantially as described.
- 45 6. In apparatus for unburdening a solvent of its load of salt, a loop formed conduit with branches in heat-exchanging relation one to the other, cooling means arranged at a point intermediate the length of the in- 50 flowing branch of the conduit, a second cooling means arranged in the loop of the conduit, and separating means arranged in the loop of the conduit beyond the cooling means last mentioned, substantially as described.
- 55 7. In apparatus for unburdening a solvent of its load of salt the combination of four heat-exchangers each including two liquid- conveying elements, four of said elements (one element of each of said heat exchangers) being connected in series and adapted to 60 convey in continuous flow an entering stream of solvent, the second element of the third and the second element of the first heat-exchanger being connected in series, in the order named, and adapted to convey in con- 65 tinuous flow the escaping stream of solvent, means for causing a separate cooling medium to circulate in the second element of the second heat-exchanger, means for causing a separate cooling medium to circulate in the 70 second element of the fourth heat exchanger, and separating apparatus adapted to receive the stream of solvent as it advances from the fourth heat-exchanger and to deliver the solvent again to the third heat-exchanger, sub- 75 stantially as described.
8. In apparatus for unburdening a solvent of its load of salt the combination of a conduit adapted to convey a body of solvent in continuous stream, means for causing a stream of liquid in part to flow over the surface of the said conduit at a higher point in the extent thereof, and in part to enter the said conduit at a lower point in the extent thereof, and means arranged at an intermediate point for separating salt from the solvent, substantially as described.
9. In apparatus for unburdening a solvent of its load of salt the combination of three heat-exchangers and a centrifuge, each heat-exchanger including two elements, three of said elements (one element of each of said heat-exchangers) being connected in series and affording a conduit for the continuous flow of the solvent and for the delivery of the entire stream to the centrifuge, means for causing a cooling medium to circulate in the second element of the third heat-exchanger, the second element of the second heat-exchanger and the second element of the first heat-exchanger being connected and affording a conduit for the return flow of the solvent issuing from the said centrifuge, sub- 95 stantially as described.
- 100 In testimony whereof we have hereunto set our hands.

HENRY S. MARSH.  
RALF S. COCHRAN.

Witnesses:

ED. J. RUSSELL,  
A. C. DAVIDSON.